# EUROPEAN PATENT SPECIFICATION

(11) **EP 0 646 187 B1**
(45) Date of publication and mention of the grant of the patent: **10.01.2001**
(21) Application number: 93914728.6
(22) Date of filing: 23.06.1993
(51) Int. Cl.: C23C 22/68, C23C 22/66, C23C 22/60, C23C 22/06

(54) **NON-CHROMATED OXIDE COATING FOR ALUMINUM SUBSTRATES**
NICHT-CHROMATIERTE OXIDÜBERZÜGE FÜR ALUMINIUMSUBSTRATE
COUCHE D'OXYDE NON CHROMATE POUR SUBSTRATS EN ALUMINIUM

(30) Priority: 25.06.1992 US 903853
(43) Date of publication of application: 05.04.1995
(73) Proprietor: THE BOEING COMPANY, Seattle, Washington 98124-2207 (US)
(72) Inventor: SCHRIEVER, Matthias, P., Kent, WA 98031 (US)
(74) Representative: Prins, Hendrik Willem
(86) International application number: EP9301630
(87) International publication number: WO9400619

(56) References cited:
- EP-A- 0 458 020
- EP-A- 0 488 430
- EP-A- 0 523 288
- US-A- 4 381 203

## Description

### Field of the Invention

This environmental-quality invention is in the field of chemical conversion coatings formed on metal substrates, for example, on aluminum substrates. More particularly, one aspect of the invention is a new type of oxide coating (which I refer to as a "cobalt conversion coating") which is chemically formed on metal substrates. The invention enhances the quality of the environment of mankind by contributing to the maintenance of air and water quality.

### Background of the Invention

In general, chemical conversion coatings are formed chemically by causing the surface of the metal to be "converted" into a tightly adherent coating, all or part of which consists of an oxidized form of the substrate metal. Chemical conversion coatings can provide high corrosion resistance as well as strong bonding affinity for paint. The industrial application of paint (organic finishes) to metals generally requires the use of a chemical conversion coating, particularly when the performance demands are high.

Although aluminum protects itself against corrosion by forming a natural oxide coating, the protection is not complete. In the presence of moisture and electrolytes, aluminum alloys, particularly of the high-copper 2000-series aluminum alloys, such as alloy 2024-T3, corrode much more rapidly than pure aluminum.

In general, there are two types of processes for treating aluminum to form a beneficial conversion coating. The first is by anodic oxidation (anodization) in which the aluminum component is immersed in a chemical bath, such as a chromic or sulfuric acid bath, and an electric current is passed through the aluminum component and the chemical bath. The resulting conversion coating on the surface of the aluminum component offers resistance to corrosion and a bonding surface for organic finishes.

The second type of process is by chemically producing a conversion coating, which is commonly referred to as a chemical conversion coating, by subjecting the aluminum component to a chemical solution, such as a chromic acid solution, but without using an electric current in the process. The chemical solution may be applied by immersion application, by manual application, or by spray application. The resulting conversion coating on the surface of the aluminum component offers resistance to corrosion and a bonding surface for organic finishes. The present invention relates to this second type of process for producing chemical conversion coatings. The chemical solution may be applied by immersion application, by various types of manual application, or by spray application.

One widely-used chromic acid process for forming chemical conversion coatings on aluminum substrates is described in various embodiments in Ostrader et al. U.S. Patent 2,796,370 and Ostrader et al. U.S. Patent 2,796,371, in military process specification MIL-C-5541, and in Boeing Process Specification BAC 5719. These chromic acid chemical conversion baths contain hexavalent chromium, fluorides, and cyanides, all of which present significant environmental as well as health and safety problems. The constituents of a typical chromic acid conversion bath, such as ALODINE 1200, are as follows: CrO₃ - "chromic acid" (hexavalent, chromium); NaF-sodium fluoride; KBF₄-potassium tetrafluoroborate; K₂ZrF₆-potassium hexafluorozirconate; K₃Fe(CN)₆ potassium ferricyanide; and, HNO₃-nitric acid (for pH control).

A process for accelerating the rate of forming conversion coatings on Zinc or Zinc alloy surfaces is taught in U.S. Patent 4381203.

Many aluminum structural parts, as well as Cd plated, Zn plated, Zn-Ni plated and steel parts, throughout the aircraft and aerospace industry, are currently being treated using this chromic acid process technology. Chromic acid conversion films, as formed on aluminum substrates, meet a 168 hours corrosion resistance criterion, but they primarily serve as a surface substrate for paint adhesion. Because of their relative thinness and low coating weights 3.72-13.84 milligrams/m² (40-150 milligrams/ft²), chromic acid conversion coatings do not cause a fatigue life reduction in the aluminum structure.

However, environmental regulations in the United States, particularly in California, and in other countries are drastically reducing the allowed levels of hexavalent chromium compounds in effluents and emissions from metal finishing processes. Accordingly, chemical conversion processes employing hexavalent chromium compounds must be replaced. The present invention, which does not employ hexavalent chromium compounds, is intended to replace the previously used chromic acid process for forming conversion coatings on aluminum substrates.

### Summary of the Invention

A. In one respect, the invention is a process for forming a cobalt conversion coating on a metal substrate, thereby imparting corrosion resistance and paint adhesion properties. The invention was developed as a replacement for the prior art chromic acid process. The process includes the steps of: (a) providing a cobalt conversion solution comprising an aqueous solution containing a soluble cobalt-III hexavalent complex, the concentration to the cobalt-III hexavalent complex being from about 0.01 mole per liter of solution to the saturation limit of the cobalt-III hexavalent complex; and (b) contacting the substrate with the solution for a sufficient amount of time, whereby the cobalt conversion coating is formed. The substrate may be aluminum, aluminum alloy, as well as Cd plated, Zn plated, Zn-Ni plated, and steel. The cobalt-III hexavalent complex is preferably present in the form of Meₘ[Co(R)₆]_{n'} wherein Me is Na, Li, K, Ca, Zn, Mg, or Mn, and wherein m is 2 or 3, n is 1 or 2, and R is a carboxylate having 1 to 6 C atoms.

B. In another aspect, the invention is a chemical conversion coating solution for producing a cobalt conversion coating on a metal substrate, the solution including an aqueous solution containing a soluble cobalt-III hexacarboxylate complex, the concentration of the cobalt-III hexacarboxylate complex being from about 0.01 mole per liter of solution to the saturation limit of the cobalt-III hexavalent complex. The cobalt conversion solution may be prepared by a bath makeup sequence including the steps of: (a) dissolving a soluble cobalt-II salt, preferably cobalt acetate, and (b) dissolving a metal acetate salt such as sodium, magnesium or calcium acetate to form a conversion coating solution.

C. In yet another aspect to the invention, wetting agents such as alkyl fluorides, fluorocarbons, and metal fluorides can be added to the conversion coating solutions. Addition of these wetting agents eliminate the need for a costly sealing step following formation of the conversion coating.

### Brief Description of the Drawings

The figures herein contained are photomicrographs of images produced by a scanning electron microscope of coatings on aluminum alloy test panels. FIGURES 1 through 4 are photomicrographs (scanning electron microscope operated at 20 KV) of alloy 2024-T3 test panels with cobalt conversion coatings made by the invention. FIGURES 1 through 4 show a cobalt conversion coatings 410 formed by a 15 minute immersion in a typical cobalt conversion coating solution at 60°C (140°F).

The foregoing aspects and many of the attendant advantages of this invention will become more readily appreciated as the same becomes better understood by reference to the following detailed description, when taken in conjunction with the accompanying drawings, wherein:

FIGURE 1 is a photomicrograph at X10,000 magnification of a test panel showing a cobalt conversation coating 410 of the invention. The photomicrograph is a top view of the upper surface of oxide coating 410. The top of oxide coating 410 is porous and looks like a sponge. This test panel was immersed in the cobalt conversion coating solution for 15 minutes. The white bar is a length of 1 micron.

FIGURE 2 is a photomicrograph at X70,000 magnification of the test panel of FIGURE 1. The photomicrograph is a top view of the upper surface of oxide coating 410. FIGURE 2 is a close-up, at higher magnification, of a small area of the test panel. The white bar is a length of 1 micron.

FIGURE 3 is a photomicron at X10,000 magnification of another test panel showing a side view, from an elevated angle, of a fractured cross section of a cobalt conversion coating 420 of the invention. The fractured cross section of the aluminum substrate of the test panel is indicated by reference numeral 422. This test panel was immersed in the coating bath for 15 minutes. To make the photomicrograph, the test panel was bent and broken off to expose a cross section of oxide coating 420. The white bar is a length of 1 micron.

FIGURE 4 is a photomicrograph at X70,000 magnification of the test panel of FIGURE 3 showing a side view, from an elevated angle, of a fractured cross section of cobalt conversion coating 420 of the invention. FIGURE 4 is a close-up, at higher magnification, of a small area of the test panel. The aluminum substrate of the test panel is indicated by reference numeral 422. The white bar is a length of 1 µm.

FIGURE 5 is a graph showing the tradeoff between paint adhesion and corrosion resistance as a function of immersion time.

### Detailed Description of the Preferred Embodiment

The present invention relates to a new cobalt conversion coating. The cobalt conversion coating can be made so resistant to corrosion that the conventional sealing step is no longer required. This result is achieved by adding metal fluorides and wetting agents such as alkyl fluorides and fluorocarbons to the conversion coating solution. It is believed that the combination of the wetting agents and the metal fluorides impart a small etch effect on the aluminum substrate surface which is believed to aid in the coating formation.

By way of background leading up to this invention, the subject matter set forth in my prior copending applications will be reviewed. A considerable amount of empirical research was conducted in order to arrive at the present invention. A variety of multivalent compounds was investigated, used either by themselves or in combination with alkalis, acids, or fluorides. Among these compounds were vanadates, molybdates, cerates, ferrates and variety of borates. While film deposition of compounds containing these elements on aluminum alloy substrates has been achieved, none afforded any appreciable corrosion protection nor paint adhesion.

Cobalt ammine complexes were thus produced with a number of reactants, i.e., Co(NO₃)• 6H₂O, CoCl₂• 6H₂O, NH₄NO₃, NH₄Cl and NH₄OH. The resultant coatings formed on aluminum substrates were found to have substantially improved corrosion resistant over the simple salt immersion described earlier. A review of cobalt complexing chemistry yielded the following information:

When a stream of air is drawn for several hours through a solution of cobalt-II salt, containing ammonium hydroxide, the corresponding ammonium salt and activated charcoal, then hexammine salts are obtained: ${\text{4 Co X}}_{\text{2}} {\text{+ 4 NH}}_{\text{4}} {\text{X + 20 NH}}_{\text{3}} {\text{+ O}}_{\text{2}} {\text{→ 4[Co(NH}}_{\text{3}} {\text{)}}_{\text{6}} {\text{] X}}_{\text{3}} \text{+ water,}$ wherein X = Cl, Br, NO₃, CN, SCN, PO₄, SO₄, C₂H₃O₂, and CO₃.
In the absence of activated charcoal, replacement will occur to give:

[Co(NH₃)₅ X]²⁺ (2)

These generic reactions are based on the fact that cobalt-II salts have a very strong tendency to oxidize to cobalt-III complexes, i.e., These reactions are not new and have been studied extensively. Cobalt-III complexes are typically made in the photo development industry as oxidizers to enhance clarity of color photography. What is surprising, however, is that cobalt complexes are capable of forming oxide structures on aluminum substrates. The exact reaction mechanism of this oxide formation is not completely understood, but is believed to function on the chemical equilibrium in Equation (3).

This oxidizing tendency is considered to be responsible for the formation of oxide films on aluminum substrates. Bath formulations were made up successfully using the following chemical balances below: ${\text{4 Co(NO}}_{\text{3}} {\text{)}}_{\text{2}} {\text{•6H}}_{\text{2}} {\text{O + 4 NH}}_{\text{4}} {\text{NO}}_{\text{3}} {\text{+ 20 NH}}_{\text{4}} {\text{OH + oxygen → 4 [Co(NH}}_{\text{3}} {\text{)}}_{\text{6}} {\text{] -NO}}_{\text{3}} {\text{)}}_{\text{3}} {\text{+ H}}_{\text{2}} \text{O}$The ammonium nitrate is used to prevent initial precipitation of the reaction products. This chemistry is extensively reviewed in EP-A-0 458 020, in the name of the inventor of the present application.

An examination of reaction (4) revealed however, that while well defined iridescent coatings could be formed on aluminum substrates, an excess of ammonia, i.e., NH₄OH was required to drive this reaction. As a consequence, it is difficult to control the pH of the bath due to the high evaporation rates of ammonia from the solution. Furthermore, the amount of excess ammonia in the bath had a pronounced effect on the paint adhesion and corrosion resistance characteristics of coatings formed by this method. Paint adhesion and corrosion performance ranged from superb to complete failure, depending on the amount of ammonia in the bath.

A major advancement of this technology was achieved when a change in the portion of the complex that includes the ligand (the bracketed portion of formula (6)) within the cobalt complex was attempted. The development of the ammoniated cobalt complexes as described under reactions (1) through (4) established the bath chemistries as 3 valent cobalt amine complexes, i.e.,

[Co(NH₃)₆]X₃ (5)

wherein X = Cl, Br, NO₃, CN, SCN, PO₄, SO₄, C₂H₃O₂, CO₃, and wherein the portion of the complex that includes the ligand is positively charged, i.e.,

[Co(NH₃)₆]³⁺ (6)

With the substitution of nitrite compounds for the ammonium compounds the formation of 3-valent cobalt complexes such as

Me₃[Co(NO₂)₆], (7)

wherein Me = Na, Li, K was achieved where the portion of the complex that includes the ligand is negatively charged, i.e.,

[Co(NO₂)₆]³⁻ (8)

This nitrite complexed chemistry was found to be completely self controlling with a stable pH in the region 6.8 to 7.2. Paint adhesion performance was also found to be substantially superior to prior chromated films. This chemistry is extensively discussed in EP-A-0 488 430 in the name of the inventor of the present application. Two pronounced characteristics of conversion films formed with this nitrite technology was the almost clear (very light iridescence) surface appearance and the coating film weights which were limited at 969 mg/m² (90 mg/ft²) maximum. These two limitations led to further research work to investigate the feasibility of obtaining coatings with strong, easily inspectable color indication along with higher coating weights, i.e., in excess of 969 mg/m² (90 mg/ft²).

Successful formulations were finally made with the introduction of acetates to form complexes such as

Me₃[Co(C₂H₃O₂)6] (9)

where the portion of the complex that includes the ligand is also negatively charged, i.e.,

[Co(C₂H₃O₂)₆]³⁻ (10)

Coatings formed by this method are strongly colored, similar to prior chromated coatings in appearance. Coating weights in excess of 3767 mg/m² (350 mg/ft²) can be achieved. Nitrates such as NaNO₃, Mg(NO₃)₂·6H₂O or Ca(NO₃)₂·6H₂O were added to this formulation to aid in coating firmness at higher coating weight thus avoiding powdery loose deposits. As a result of this research, two bath formulations that resulted in a clear coating and a colored coating were selected for further testing. The following two equations below establish the chemistries for the clear and colored cobalt conversion coatings.

Clear Coat: ${\text{Co(NO}}_{\text{3}} {\text{)}}_{\text{2}} {\text{·6H}}_{\text{2}} {\text{O + 6NaNO}}_{\text{2}} {\text{+ 1/2H}}_{\text{2}} {\text{O}}_{\text{2}} {\text{→ Na}}_{\text{3}} {\text{[Co(NO}}_{\text{2}} {\text{)}}_{\text{6}} {\text{] + 2NaNO}}_{\text{3}} \text{+ 2NaOH}$

Colored Coat: ${\text{Co(NO}}_{\text{3}} {\text{)}}_{\text{2}} {\text{• 6H}}_{\text{2}} {\text{O + 6CH}}_{\text{3}} {\text{COONH}}_{\text{4}} {\text{1/2H}}_{\text{2}} {\text{O}}_{\text{2}} {\text{→ Na}}_{\text{3}} {\text{[Co(C}}_{\text{2}} {\text{H}}_{\text{3}} {\text{O}}_{\text{2}} {\text{)}}_{\text{6}} {\text{] + 2NH}}_{\text{4}} {\text{NO}}_{\text{3}} {\text{+ NH}}_{\text{4}} \text{OH}$When coatings are produced by equations (11) and (12) and are sealed subsequently in special formulated solutions, up to 140 hours of salt spray corrosion resistance are obtained when tested in accordance with ASTM B 117. This chemistry is extensively discussed in EP-A-0 523 288, in the name of the inventor of the present application.

The research advances described up to this point involve conversion coatings formed from the reaction of a 2-valent cobalt salt such as Co(NO₃)₂• 6H₂O with ammonium acetate (CH₃COONH₄) to form a 3-valent cobalt complex. The resultant coatings are of superb quality with regard to defined performance criteria; however, the bath life of solutions utilizing ammonium acetate are rather short, i.e., on the order of 30 to 40 days. The desire to extend this bath life was the basis for further research that was just recently completed. This work has now progressed to overall process and coating performance improvements in accordance with the present invention, as discussed in further detail below.

During testing of the ammonium acetate complexed cobalt solution (Equation (12)), it was noticed that after several weeks of normal tank operation the coating weights on aluminum substrates would gradually drop off and the color intensity would become lighter. In order to compensate for this, ever increasing immersion times were required. It was also noticed that a gradual solution appearance change would occur over time, from a dark brown to wine red color Analysis finally established that a competing reaction was taking place over time, where the acetate in the complex

[Co(C₂H₃O₂)₆]³⁻ (13)

would gradually be replaced by an ammonia to form the complex

[Co(NH₃)₆]³⁺ (14)

Notice the valence change in these bracketed ionic species.

In an effort to solve this problem it was discovered, in accordance with the present invention, that the substitution of a metal acetate such as Na(C₂H₃O₂)• 3H₂O, Mg(C₂H₃O₂)₂ • 4H₂O, or Ca(C₂H₃O₂)₂ • H₂O for the NH₄(C₂H₃O₂) in Equation (12) would eliminate the above competing reactions described in conjunction with complexes (13) and (14), and result in the same strong colored coatings as the original ammonium acetate solutions. Sodium acetate is the most preferred metal carboxylate. Other metal carboxylates such as zinc, lithium, potassium, and manganese acetate will work but are not preferred. The typical reactions are ${\text{2Co(C}}_{\text{2}} {\text{H}}_{\text{3}} {\text{O}}_{\text{2}} {\text{)}}_{\text{2}} {\text{• 4H}}_{\text{2}} {\text{O + 3 Mg(C}}_{\text{2}} {\text{H}}_{\text{3}} {\text{O}}_{\text{2}} {\text{)}}_{\text{2}} {\text{• 4H}}_{\text{2}} {\text{O +2HC}}_{\text{2}} {\text{H}}_{\text{3}} {\text{O}}_{\text{2}} {\text{→ Mg}}_{\text{3}} {\text{[Co(C}}_{\text{2}} {\text{H}}_{\text{3}} {\text{O}}_{\text{2}} {\text{)}}_{\text{6}} {\text{]}}_{\text{2}} {\text{+ 21H}}_{\text{2}} \text{O}$${\text{Co(C}}_{\text{2}} {\text{H}}_{\text{3}} {\text{O}}_{\text{2}} {\text{)}}_{\text{2}} {\text{• 4H}}_{\text{2}} {\text{O + 3Ca(C}}_{\text{2}} {\text{H}}_{\text{3}} {\text{O}}_{\text{2}} {\text{)}}_{\text{2}} {\text{• H}}_{\text{2}} {\text{O +1/2 O}}_{\text{2}} {\text{+ 2HC}}_{\text{2}} {\text{H}}_{\text{3}} {\text{O}}_{\text{2}} {\text{→ Ca}}_{\text{3}} {\text{[Co(C}}_{\text{2}} {\text{H}}_{\text{3}} {\text{O}}_{\text{2}} {\text{)}}_{\text{6}} {\text{]}}_{\text{2}} {\text{+ 21H}}_{\text{2}} \text{O}$${\text{Co(C}}_{\text{2}} {\text{H}}_{\text{3}} {\text{O}}_{\text{2}} {\text{)}}_{\text{2}} {\text{• 4H}}_{\text{2}} {\text{O + 3Na(C}}_{\text{2}} {\text{H}}_{\text{3}} {\text{O}}_{\text{2}} {\text{) • 3H}}_{\text{2}} {\text{O + 1/4O}}_{\text{2}} {\text{+ HC}}_{\text{2}} {\text{H}}_{\text{3}} {\text{O}}_{\text{2}} {\text{→ Na}}_{\text{3}} {\text{[Co(C}}_{\text{2}} {\text{H}}_{\text{3}} {\text{O}}_{\text{2}} {\text{)}}_{\text{6}} {\text{] + 13 1/2H}}_{\text{2}} \text{O}$

These reactions are carried out by bubbling air through the solution without the use of hydrogen peroxide. The acetic acid is not added as a reactant, but is formed in solution as part of the complex chemical reaction. The resultant conversion coatings are further improved in corrosion resistance over those conversion coating solutions produced by the reactions of Equations (11) and (12) when subjected to salt spray testing per ASTM B117. In the broader context, it has been found that a cobalt conversion coating having superior performance characteristics can be produced by reacting a soluble cobalt salt with a metal carboxylate in accordance with the following general formula ${\text{Soluble Cobalt Salt + Me(R)}}_{\text{x}} {\text{→Me}}_{\text{m}} {\text{[Co(R)}}_{\text{6}} {\text{]}}_{\text{n}} \text{,}$wherein x can be 1 or 2, m is 3, n is 1 or 2, Me is selected from the group consisting of Na, Li, K, Ca, Zn, Mg, and Mn, and wherein R is a carboxylate having from 1 to 5 carbon (C) atoms, provided the carboxylates are soluble in the reaction solution.

Metal fluorides such as MgF₂ and CaF₂ and wetting agents such as water soluble alkyl-fluorides and fluorocarbons can also be added in very small quantities to these solutions (Tables III and IV) to improve corrosion protection and manufacturing ease. In particular alkyl fluoride wetting agents such as MSP-ST alkyl fluoride by M&T Harshaw, Cleveland, Ohio, and fluorocarbons FC99 or FC95 wetting agents by 3M Company, St. Paul, Minnesota, have been successfully used. The presence of the fluorinated wetting agents, metal fluorides, or mixtures thereof raise the corrosion performance level of resultant coatings to such a degree that sealing of these conversion coatings in a secondary seal step is no longer required. In principle any water soluble fluorinated wetting agent capable of lowering liquid surface tension into the range of 0.03 N/m to 0.04 N/m (30 to 40 dynes per centimeter) at 20°C is usable. Solutions operated as detailed below yield coatings that pass a 168 hours salt spray corrosion resistance criteria in accordance with Boeing Process Specification BAC 5719, "Chromated Conversion Coatings." The single step conversion coating has 'yielded in excess of 240 hours of salt spray resistance before showing any sign of corrosion pitting.

It became apparent during experimentation with formulations (16), (17) and (18) that certain parameters are critical with respect to both make-up, chemistry and consistency of coating performance. These parameters were found to be bath makeup and process sequence, reactant selection and bath concentrations, temperature control, and immersion times. It must also be emphasized that the reaction system created is very complex and involves several simultaneous reversible reactions. It is believed that the entire reaction system must be present at or near an equilibrium condition in order to achieve optimum results in accordance with the present invention.

### Reactant Selection Concentrations

The most critical parameters affecting performance of conversion coatings with respect to paint adhesion and corrosion resistance were found to be selection of the reactants and their concentrations in solution. It was found that coating performance was affected foremost by these factors rather than bath temperature or immersion time do impact their effects over lager variations of these parameters.

It is known that with respect to surface treatments of aluminum, paint adhesion and corrosion resistance are divergent properties. In other words, maximizing paint adhesion usually occurs at the expense of corrosion performance and vice-versa. This surface treatment behavior was also found to exist with cobalt conversion coatings. The research carried out and described in this and the aforementioned prior copending applications has established a preferential list with regard to the various cobalt compounds and their corrosion resistance effectiveness versus paint adhesion.

**TABLE I -**

| Performance Rating of Cobalt Salts Using Metal Acetates for Complexing | | |
|---|---|---|
| Component | Corrosion Resistance | Paint Adhesion |
| Cobalt Acetate + Me Acetate | 1 | 2 |
| Cobalt Nitrate + Me Acetate | 3 | 1 |
| Cobalt Sulfate + Me Acetate | 2 | 4 |
| Cobalt Chloride + Me Acetate | 4 | 3 |
| Rating: 1 = best, 4 = worst | | |

It can be seen from Table I that the cobalt acetate formulations present the best possible combination with respect to corrosion resistance while maintaining good paint adhesion performance. It should be noted, however, that in cases where corrosion performance is not a factor, nitrates or nitrites yield the best paint adhesion performance that is achievable with these cobalt complexed salts.

Cobalt acetate is the most preferred soluble cobalt-II salt. Other water soluble cobalt salts such as Co(NO₃)₂, CoSO₄, CoCl_{2,} CoPO₄, CoCO₃, may be substituted for cobalt acetate, but are not preferred for the reasons illustrated in Table I. These cobalt salts are preferably reacted with soluble metal carboxylates having from 1 to 5 carbon atoms, although metal salts of acetic acid are most preferred. The carboxylate salts of Ca, Mg, and Na are preferred, with the Na carboxylate being most preferred, while Zn, Li, K, and Mn may also be used. The limitations on using carboxylates other than the acetates is water solubility. Other carboxylates that will work are for example sodium propionate. The minimum solubility needed to produce an effective coating is about 0.01 moles of cobalt-II salt per liter of water at 20°C. (68°F). The salts may be used up to their solubility limits.

Although not required, fluorinated wetting agents may be added to the bath as discussed above. When these wetting agents are employed, a conversion coating is created that does not need to be subjected to a conventional sealing step in order to exhibit satisfactory corrosion resistance.

### Chemical Concentration, pH Control, Temperature, and Immersion Time

With respect to chemical concentrations, the concentration of dissolved cobalt-II salt used may be from about 0.01 mole per liter of final solution up to the solubility limit of the cobalt-II salt employed at 20°C (68°F). Preferably, the concentration of dissolved cobalt-II salt used may be from about 0 04 mole per liter of final solution up to 0.15 mole per liter of final solution.

The concentration of the cobalt-III hexcarboxylate coordination complex may be from about 0.01 mole per liter of final solution up to the solubility limit of the cobalt-III hexcarboxylate coordination complex employed. Preferably , the concentration of the cobalt-III hexcarboxylate coordination complex may be from about 0.04 mole per liter of final solution up to 0.15 mole per liter of final solution.

The concentration of dissolved metal carboxylate, preferably a metal acetate, may be from about 0.03 to 2.5 moles per liter of final solution. Preferably, the concentration of dissolved metal carboxylate used may be from about 0.05 mole per liter of final solution up to 0.2 mole per liter of final solution.

When employed, the concentration of the fluorinated wetting agents is preferably sufficient to hold solution surface tension between 3x10⁻⁶ Nm to 4x10⁻⁶ Nm (30 to 40 dynes) per centimeter at 20°C. The metal fluorides, MgF₂ and CaF₂, may be present in a concentration from 0 to solubility limit. It is to be understood that the fluorinated wetting agents, metal fluorides, or mixtures thereof are not required, but are preferred. If the wetting agents and metal fluorides are not used, the conversion coating must be subjected to a sealing step to achieve high corrosion resistance. By using the wetting agents and fluorides, the sealing step can be eliminated, thus making the use of the present invention even more economical.

The pH of the bath may be from about 5.0 to 9.0 with 6.0 to 7.5 being preferred and 6.5 being most preferred. The temperature of the bath may be from about 20°C to 71,1°C (68°F to 160°F). Above 71,1°C (160°F), gradual decomposition of the cobalt-III hexcarboxylate complex may occur. The optimum temperature is 60±2.2°C (140±5°F). The immersion time may be from about 3 minutes to 60 minutes, more preferably from 5 to 30 minutes. When sodium acetate is employed, the immersion time can be reduced to 5 to 8 minutes. Use of these parameters will result in coating weights ranging for example from 215 mg/m² to 2583 mg/m² (20 to 240 mg/ft²).

### Preferred Bath Preparation Sequence

The following bath make up sequence is preferred for the acetate complexed cobalt solution:
1. A stainless steel tank is equipped with air agitation and temperature control equipment capable of controlling temperature within ±22°C (±5°F). (The tank may be lined with an inert material capable of withstanding 65.5°C (150°F) continuous operation.)
2. The tank is filled to 3/4-full with deionized water and heated to 48.8°C (120°F). Air agitation is commenced to achieve a gentle boil.
3. The applicable amount of metal acetate salt is now added and dissolved. For larger tanks a fine meshed holding basked will serve as a holding device aiding in the dissolution of the material.
4. The applicable amount of cobalt salt is then added and dissolved. A gentle air boil of the tank solution is maintained for another four hours at which time the reaction is mostly completed. A holding basket may also be used to aid in dissolution.
5. The solution is now heated to 60°C (140°F) and the required small amounts of fluorinated wetting agent are added. Air agitation is maintained for an additional two hours. The tank is now ready for operation.

### Preferred Overall Processing Sequence

The preferred overall processing sequence may be summarized as follows:
1. Preclean
2. Mask and Rack
3. Alkaline Clean
4. Rinse at Room Temperature
5. Deoxidize
6. Rinse at Room Temperature
7. Form Oxide Conversion Coating
8. Rinse at Room Temperature
9. Dry

### General Notes With Respect To The Above Process Flow Charts

The cobalt conversion coating should be applied after all trimming and fabrication have been completed. Parts, where solution entrapment is possible, should not be subjected to immersion alkaline cleaning or immersion deoxidizing; manual cleaning and manual deoxidizing procedures should be used to obtain water break-free surfaces before applying cobalt conversion treatment. A water break-free surface is a surface which maintains a continuous water film for a period of at least 30 seconds after having been sprayed or immersion rinsed in clean water at a temperature below 37.7°C (100°F).

Thorough rinsing and draining throughout processing is necessary as each solution should be completely removed to avoid interference with the performance of the next solution in the sequence. Parts should be processed from one step to the next without delay and without allowing the parts to dry. When it is necessary to handle wet parts, clean latex rubber gloves should be worn. After conversion coating, handle dry parts only with clean fabric gloves. For processing systems which require part clamping, the number and size i of contact points should be kept to a minimum as necessary for adequate mechanical support.

### Preclean

Vapor degrease may be performed in accordance with Boeing Process Specification BAC 5408. Emulsion clean in accordance with Boeing Process Specification BAC 5763, or solvent clean in accordance with Boeing Process Specification BAC 5750 if parts are greasy or oily. Parts with open faying surfaces or spot-welded joints where solution entrapment is possible should be immersed in cold water (or in hot and cold water) for 2 minutes after precleaning.

### Mask and Rack

Areas which do not require cobalt conversion coatings should be masked with maskants. Dissimilar metal inserts (except chromium, nickel or cobalt alloy or plating, CRES, or titanium) and non-aluminum coated plasma flame sprayed area should be masked off. Parts are then racked in holding baskets or mounted on holding fixtures.

### Alkaline Clean

Alkaline clean and rinse may be performed in accordance with Boeing Process Specification BAC 5749, except for parts with open faying surfaces or spot welded joints, in which case, rinsing should be for at least 10 minutes using agitation with multiple immersions (a minimum of four times) followed by manual spray rinsing as required to prevent solution entrapment.

### Deoxidize

Deoxidize and rinse may be performed in accordance with Boeing Process Specification BAC 5765 except for parts where solution entrapment is possible, which parts may be rinsed using the method described above under "Alkaline Cleaning". Castings may be deoxidized by either of the following methods:
a. Deoxidize in accordance with Boeing Process Specification BAC 5765, Solution 37, 38 or 39.
b. Dry abrasive blast castings in accordance with Boeing Process Specification BAC 5748, Type II, Class 1 and rinse.

A specific solution formulation within the scope of the invention is as set forth in TABLE II, below.

**TABLE II**

| Preferred Solution Formulation | | |
|---|---|---|
| Component¹ | Makeup Per Liter | Control Range |
| Cobalt Acetate Co(C₂H₃O₂)₂•4H₂O | 33.0 g | 30 - 35 g |
| Magnesium Acetate Mg(C₂H₃O₂)₂•4H₂O | 85.0 g | 80 - 90 g |
| or | | |
| Calcium Acetate Ca(C₂H₃O₂)₂•H₂O | 70.0 g | 65 - 75 g |
| or | | |
| Sodium Acetate Na(C₂H₃O₂)•H₂O | 125.0 g | 120-130 g |
| Alkyl-Fluoride (MSP-ST) | 4-5 ml | ² |
| Magnesium Fluoride MgF₂ | 2 g | 1-3 g |
| or | | |
| Calcium Fluoride CaF₂ | 2 g | 1-3 g |
| Operating Temperature | 37.7°C (100°F) (Makeup) | 57.2-62.7°C (135-145°F) Operation) |
| Immersion Time | | 5-20 min. (5 to 8 Min for Na Acetate) |

| | | |
|---|---|---|
| ¹ Coatings formed with this technology do not require sealing for corrosion resistance. | | |
| ² Maintain solution surface tension between 3 to 4 µN/m (30 to 40 dynes per centimeter). | | |

Bath temperature variations and immersion times also contribute to corrosion performance and paint adhesion, however, to a significantly lesser degree than the solution reactant selection. It was determined that the variations in both temperatures and immersion time will affect the coating thickness primarily, while the reactant materials primarily influence coating structure and density. The following general performance effects were observed:
1. Optimum bath temperature from the standpoint of corrosion and adhesion was found to be 60°C ± 2.2°C (140°F ± 5°F).
2. An increase in bath temperature from optimum does result in thick and looser coatings and thus a decrease in paint adhesion with an increase in corrosion resistance.
3. A decrease in bath temperature from optimum results in thinner coatings with an increase in paint adhesion and a decrease in corrosion resistance.
4. The optimum time was found to be a function of reactant selection.
5. For nitrite complexed cobalt salts the optimum > immersion time was 20-25 minutes at optimum bath temp.
6. For acetate complexed cobalt salts the optimum immersion was found to be a function of the type of acetate being used, i.e.
   For Na(C₂H₃O₂) 5 - 8 min at 60°C (140°F)
   For Mg(C₂H₃O₂)₂ 15 - 20 min at 60°C (140°F)
   For Ca(C₂H₃O₂)₂ 12 - 15 min at 60°C (140°F)

FIGURE 5 depicts the general behavior of cobalt conversion coatings with respect to corrosion performance vs. paint adhesion. The intercept point of the corrosion and adhesion curve represents the bath parameters where the two divergent properties (corrosion and adhesion) are at optimum with respect to each other.

It is preferred that the pH be maintained between pH 6.0 and 7.5, although coatings have been produced between pH 5.0 and 9.0. Adjustments to the pH may be required after the solutions have been used for extended periods.

### Corrosion Resistance

Utilizing the basic corrosion resistance behavior of complexed cobalt salts, as shown above, the cobalt acetate formulations were investigated extensively. Cobalt acetate was complexed with sodium acetate Na(C₂H₃O₂) ·3H₂O or magnesium acetate Mg(C₂H₃O₂)₂·4H₂O. The results show that these formulations have excellent corrosion resistance without a subsequent seal step. Salt spray corrosion testing was conducted in accordance with ASTM B117 and all specimens were subjected to 168 hr. exposure. See Tables III and IV for results. The test conditions were repeated two more times and near identical results to Tables III and IV were obtained. Analysis of this data in conjunction with basic paint adhesion data, as well as other solution maintenance parameters has resulted in the optimum tank makeup and controls as listed under Table II, above. A final question on corrosion performance and color iridescence was answered with this work. This research established why sodium acetate Na(C₂H₃O₂)•3H₂O was chosen as the most preferred complexer over magnesium acetate Mg(C₂H₃O₂)₂ • 4H₂O. The reason is that sodium acetate imparts a somewhat more aggressive etch effect on the aluminum substrate. This by itself was found to be very detnmental to corrosion performance. However, when sodium acetate was chemically formulated with wetting agents and metal fluorides, it had the distinct advantage that bright color iridescence of coatings were maintained while corrosion resistance was not impaired. On the other hand, when magnesium acetate or calcium acetate were utilized in conjunction with the wetting agents and metal fluorides very little etch effect was imparted and resultant coatings were rather weak in color effect.

**Table III**

| Salt Spray Corrosion Testing of Cobalt Complex Formulations To ASTM B117 - Single Step Immersion - No Seal | | | |
|---|---|---|---|
| Component | Bath Temp Deg.°C (Deg.°F) | Immersion Time (minutes) | Salt Spray Corrosion Resistance (168 hrs. ASTM B117 |
| | | | |
| Co(C₂H₃O₂)•6H₂O and Na(C₂H₃O₂)•3H₂0 complexed | 48.8 (120) | 5 | fail |
| | 48.8 (120) | 10 | fail |
| | 48.8 (120) | 15 | fail |
| | 48.8 (120) | 20 | marginal |
| plus | 60 (140) | 5 | pass |
| MgF₂ and | 60 (140) | 10 | pass |
| Alkyl-fluoride (MSP-ST) | 60 (140) | 15 | pass |
| | 60 (140) | 20 | pass |
| | 65.5 (150) | 5 | pass |
| | 65.5 (150) | 10 | pass (powdery coat) |
| | 65.5 (150) | 15 | pass (powdery coat) |
| | 65.5 (150) | 20 | pass (powdery coat) |
| Co(C₂H₃O₂)₂•6H₂O and Mg(C₂H₃O₂)2•4H₂O complexed | 48.8 (120) | | |
| | 48.8 (120) | 5 | fail |
| | 48.8 (120) | 10 | fail |
| | 48.8 (120) | 15 | fail |
| | 48.8 (120) | 20 | fail |
| plus | 60 (140) | 5 | pass stained |
| MgF₂ and | 60 (140) | 10 | pass stained |
| Alkyl-fluoride (MSP-ST) | 60 (140) | 15 | pass stained |
| | 60 (140) | 20 | pass stained |
| | 65.5 (150) | 5 | pass stained |
| | 65.5 (150) | 10 | pass stained |
| | 65.5 (150) | 15 | pass stained |
| | 65.5 (150) | 20 | pass stained |
| Control ALODINE 1200S (current chromated system) | BAC 5719 | | pass |

**Table IV**

| Paint Adhesion Test Results on BMS 10-11¹ Paint System | | | | | |
|---|---|---|---|---|---|
| Component | Bath Temp Deg. °C (Deg. °F) | Immersion Time | BMS 10-11 Coating | Wet | Dry |
| Co(C₂H₃O₂)•6H₂O and | 48.8. (120) | 20 | TYPE I | 10 | 10 |
| Mg(C₂H₃O₂)₂•4H₂O | 48.8 (120) | 20 | TYPE I & II | 10 | 10 |
| complexed | 48.8 (120) | 30 | TYPE I | 10 | 10 |
| | 48.8 (120) | 30 | TYPE I & II | 9 | 10 |
| | 60 (140) | 20 | TYPE I | 10 | 9 |
| | 60 (140) | 20 | TYPE I & II | 9 | 10 |
| | 60 (140) | 30 | TYPE I | 10 | 10 |
| | 60 (140) | 30 | TYPE I & II | 9 | 10 |
| Co(C₂H₃O₂)₂•6H₂O | 48.8 (120) | 10 | TYPE I | 10 | 10 |
| Na(C₂H₃O₂)•3H₂O | 48.8 (120) | 10 | TYPE I & II | 10 | 10 |
| completed | 48.8 (120) | 15 | TYPE I | 9 | 10 |
| | 48.8 (120) | 15 | TYPE I & II | 9 | 10 |
| | 60 (140) | 10 | TYPE I | 10 | 10 |
| | 60 (140) | 10 | TYPE I & II | 10 | 10 |
| | 60 (140) | 15 | TYPE I | 9 | 9 |
| | 60 (140) | 15 | TYPE I & II | 9 | 9 |
| Control | BAC 5719 OR | | TYPE I | 9 | 10 |
| ALODINE 1200S | MIL-C-5541 | | TYPE I & II | 9 | 10 |
| Rating: 10 = Best 1 = Worst TYPE I - Chromated epoxy primer (aircraft high-performance coating) TYPE II - Non-chromated epoxy enamel topcoat (aircraft high performance coating) | | | | | |

| | | | | | |
|---|---|---|---|---|---|
| ¹ Boeing Material Specification BMS 10-11 is a highly cross-linked epoxy primer system and details the performance requirements of these coatings. | | | | | |

### Oxide Coating Analyses

ESCA surface analysis, using a Perkin-Elmer Model 550 surface analyzer, and Auger oxide profiles, using the same machine (in a different operating mode), have been performed in order to characterize the cobalt conversion coatings of the invention. (ESCA = electron spectroscopy for chemical analysis (also known as XPS or X-ray photoelectron spectroscopy).) These analyses show that the cobalt conversion coating consists of a mixture of oxides, namely, aluminum oxide AL₂O₃ as the largest volume percent, and cobalt oxides CoO, Co₂O₃, and Co₃O₄ Al₂O₃. The term "largest volume percent" means that the volume of this oxide exceeds the volume of any other oxide which is present, but the term "largest volume percent" means that the volume of this oxide exceeds the volume of any other oxide which is present, but the term "largest volume present" does not necessarily imply that the volume of this oxide is more than 50 volume percent.

The data further shows that in the lower portion of the oxide coating (that is, next to the aluminum substrate), the largest volume percent is AL₂O₃. The middle portion of the oxide coating is a mixture of CoO, Co₂O₃, Co₃O₄, and Al₂O₃. And the data shows that in the top portion of the oxide coating, the largest volume percent is a mixture of co₂O₃ and Co₃O₄.

Additional characterization of the cobalt conversion coatings of the invention may be found in FIGS. 1 through 4 and in the descriptions of FIGS. 1 through 4 above. FIGS. 1 through 4 show a cobalt conversion coating 410 and 420 formed by a 15 minute immersion in a typical cobalt conversion coating solution. The top surface of the cobalt conversion coating, as shown in FIGS. 1 through 4 bears a resemblance to a sponge, thus providing substantial surface area and porosity for good paint adhesion. Below the top surface, the coating becomes more dense and solid (nonporous).

### Other Method of Application

The above formulation illustrates producing cobalt conversion coatings by immersion application. The same principles apply to producing the conversion coating by manual application and by spray application.

As will be apparent to those skilled in the art to which the invention is addressed, the present invention may be embodied in forms other than those specifically disclosed above, without departing from the essential characteristics of the invention. The particular embodiments of the invention described above and the particular details of the processes described are therefore to be considered in all respects as illustrative and not restrictive. The scope of the present invention is as set forth in the appended claims rather than being limited to the examples set forth in the foregoing description. Any and all equivalents are intended to be embraced by the claims.

## Claims

1. A process for forming an oxide film cobalt conversion coating on a substrate, wherein said substrate is aluminum or aluminum alloy, said process comprising the steps of:
(a) providing an oxide film forming cobalt conversion solution comprising an aqueous reaction solution comprising a soluble cobalt-III hexacoordinated complex, where said cobalt-III hexacoordinated complex is present in the form of Meₘ[Co(R)₆]ₙ, wherein Me is one or more selected from the group consisting of Na, Li, K, Ca, Zn, Mg and Mn, and wherein m is 2 or 3, n is 1 or 2, and R is a carboxylate having from 1 to 5 C atoms, the concentration of said cobalt-III hexacoordinated complex being from about 0.01 mole per liter of said aqueous reaction solution up to the saturation limit of said cobalt-III hexacoordinated complex; and
(b) contacting said substrate with said aqueous reaction solution for a sufficient amount of time to oxidize the surface of said substrate, whereby said oxide film cobalt conversion coating is formed, wherein said aqueous reaction solution has a pH of about 5.0 to 9.0.

2. The process of claim 1 wherein an alkyl fluoride or fluorocarbon wetting agent is added to said aqueous reaction solution in the amount required to produce a liquid surface tension of 0.03 N/m to 0.04 N/m (30 to 40 dynes per centimeter).

3. The process of claims 1 or 2, wherein R is acetate.

4. The process of claims 1, 2 or 3, wherein the concentration of said cobalt-III hexavalent complex is from about 0.04 mole per liter of solution up to about 0.15 mole per liter of solution.

5. The process according to any of the claims 1-4, wherein said cobalt conversion solution is provided by reacting a cobalt-II salt with a metal carboxylate having from 1 to 5 carbon atoms.

6. The process of claim 5, wherein the concentration of said cobalt-II salt is from about 0.04 mole per liter of final solution up to about 0.15 mole per liter of final solution, and the concentration of metal carboxylate is from about 0.03 to 2.5 mole per liter of final solution.

7. The process of claims 5 or 6, wherein said cobalt-II salt is a cobalt-II salt which has a minimum solubility of about 0.01 moles of cobalt-II salt per liter of water at 20°C (68°F).

8. The process according to any of the claims 5-7, wherein said cobalt-II salt is cobalt acetate.

9. The process of claim 5, wherein said cobalt conversion solution is prepared by a bath makeup sequence comprising:
(a) dissolving said metal carboxylate salt, and
(b) then adding said cobalt-II salt.

10. The process of claim 1, wherein said cobalt conversion solution has a pH of about 5.0 to 9.0.

11. The process of claim 1, wherein said cobalt conversion solution has a temperature of about 20°C to 71.1°C (68°F to 160°F).

12. The process of claim 1, wherein said substrate is contacted with said cobalt conversion solution for a time of about 3 minutes to 60 minutes.

13. The process of claim 1, wherein a fluorinated wetting agent is added to said cobalt conversion solution to assist in the formation of said cobalt conversion coating on said substrate.

14. The process of claim 13, wherein said wetting agent is selected from the group comprising alkyl fluoride, fluorocarbons, CaF₂, MgF₂, and mixtures thereof.

15. The process of claim 13, wherein said wetting agent is added in the amount required to produce a liquid surface tension of 0.03 to 0.04 N/m (30 to 40 dynes per centimeter).

16. The process of claim 13, wherein MgF₂, CaF₂ or mixtures thereof are added to said solution in an amount ranging from 2 to 4 grams per liter of final solution.

17. The process of claim 1, wherein said substrate is aluminum, aluminum alloy, magnesium, magnesium alloy, Cd plated substrate or a Zn-Ni plated substrate.

18. An article produced by the process of claim 1.

19. A chemical conversion coating solution for producing an oxide film cobalt conversion coating on a metal substrate, said solution comprising an aqueous reaction solution comprising a soluble cobalt-III hexacoordinated complex present in the form of Meₘ[Co(R)₆]ₙ wherein Me is one or more selected from the group consisting of Na, Li, K, Ca, Zn, Mg and Mn, and wherein m is 2 or 3, n is 1 or 2, and R is a carboxylate having from 1 to 5 C atoms, the concentration of said cobalt-III hexacoordinated complex being from about 0.01 mole per liter of solution to the saturation limit of said cobalt-III hexacoordinated complex, the aqueous reaction solution having a pH of about 5.0 to 9.0.

20. The solution of claim 19, wherein R is acetate.

21. The solution of claim 19, wherein said soluble cobalt-III hexacoordinated complex is a soluble cobalt-III carboxylate complex obtainable by reacting a cobalt-II salt with a metal carboxylate salt wherein the Metal Me is defined in claim 19 having from 1 to 5 C atoms.

22. The solution of claim 21, wherein the concentration of said cobalt-II salt is from about 0.01 mole per liter of final solution up to the saturation limit of the cobalt-II salt employed, and the concentration of said metal carboxylate salt is from about 0.03 to 2.5 mole per liter of final solution.

23. The solution of claim 21, wherein said cobalt-II is a cobalt-II salt is a cobalt-II salt which has a minimum solubility of about 0.01 mole of cobalt-II salt per liter of water at 20°C (68°F).

24. The solution of claim 21, wherein said cobalt-II salt is cobalt acetate.

25. The solution of claim 21, wherein said metal carboxylate is a metal acetate.

26. The solution of claim 21, wherein said cobalt conversion solution is prepared by a bath makeup sequence comprising:
(a) dissolving said metal carboxylate; and
(b) then adding said cobalt-II salt.

27. Use of the solution of claim 19, for producing an oxide film cobalt conversion coating on a metal substrate, wherein said solution has a pH of about 5.0 to 9.0

28. Use of the solution of claim 19 for producing an oxide film cobalt conversion coating or a metal substrate, wherein said solution has a temperature of about 20°C to 71.7°C (68°F to about 160°F)

29. Use of the solution according to claim 19 for producing an oxide film cobalt conversion coating on a metal substrate, wherein said substrate is aluminum, aluminum alloy, magnesium, magnesium alloy, Cd plated substrate or a Zn-Ni plated substrate.

30. The solution of claim 19, comprising a fluorinated wetting agent added to said cobalt conversion solution to assist in the formation of said cobalt conversion coating on said substrate.

31. The solution of claim 30, wherein said wetting agent is selected from the group comprising alkyl fluoride, fluorocarbons, CaF₂, MgF₂, and mixtures thereof.

32. The solution of claim 30, wherein said wetting agent is added in the amount required to produce a liquid surface tension of 0.03 to 0.04 N/m (30 to 40 dynes per centimeter).

33. The solution of claim 30, wherein MgF₂, CaF₂ or mixtures thereof are added to said solution in an amount ranging from 2 to 4 grams per liter of final solution.

## Patentansprüche

1. Verfahren zum Ausbilden einer Oxidfilmcobaltkonversionsbeschichtung auf einem Substrat, worin das Substrat Aluminium oder eine Aluminiumlegierung ist, wobei das Verfahren die folgenden Schritte umfaßt:
(a) Vorsehen einer einen Oxidfilm bildenden Cobaltkonversionslösung, umfassend eine wäßrige Reaktionslösung, die einen lösbaren Cobalt-III-hexakoordinierten Komplex enthält, wobei der Cobalt-III-hexakoordinierte Komplex in der Form von Meₘ[Co(R)₆]ₙ vorhanden ist, worin Me eines oder mehrere ist bzw. sind, das bzw. die aus der aus Na, Li, K, Ca, Zn, Mg und Mn bestehenden Gruppe ausgewählt ist bzw. sind und worin m 2 oder 3 ist, n 1 oder 2 ist und R ein Carboxylat ist, das 1 bis 5 C-Atome hat, wobei die Konzentration des Cobalt-III-hexakoordinierten Komplexes von etwa 0,01 Mol pro Liter der wäßrigen Reaktionslösung bis zu der Sättigungsgrenze des Cobalt-III-hexakoordinierten Komplexes ist; und
(b) Kontaktieren des Substrats mit der genannten wäßrigen Reaktionslösung während eines genügenden Betrags an Zeit zum Oxidieren der Oberfläche des Substrats, wodurch die Oxidfilmcobaltkonversionsbeschichtung ausgebildet wird, wobei die wäßrige Reaktionslösung einen pH von etwa 5,0 bis 9,0 hat.

2. Verfahren nach Anspruch 1, worin ein Alkylfluorid- oder Fluorkohlenstoffbenetzungsmittel zu der wäßrigen Reaktionslösung in der Menge hinzugefügt wird, die erforderlich ist, um eine Flüssigkeitsoberflächenspannung von 0,03 N/m bis 0,04 N/m (30 bis 40 Dyne pro Zentimeter) zu erzeugen.

3. Verfahren nach Anspruch 1 oder 2, worin R Acetat ist.

4. Verfahren nach Anspruch 1, 2 oder 3, worin die Konzentration des Cobalt-III-hexavalenten Komplexes von etwa 0,04 Mol pro Liter der Lösung bis zu etwa 0,15 Mol pro Liter der Lösung beträgt.

5. Verfahren gemäß irgendeinem der Ansprüche 1 bis 4, worin die Cobaltkonversionslösung durch Reagieren eines Cobalt-II-Salzes mit einem Metalcarboxylat, das 1 bis 5 Kohlenstoffatome hat, vorgesehen wird.

6. Verfahren nach Anspruch 5, worin die Konzentration des Cobalt-II-Salzes von etwa 0,04 Mol pro Liter der endgültigen Lösung bis zu etwa 0,15 Mol pro Liter der endgültigen Lösung ist und die Konzentration des Metallcarbocylats von etwa 0,03 bis 2,5 Mol pro Liter der endgültigen Lösung beträgt.

7. Verfahren nach Anspruch 5 oder 6, worin das Cobalt-II-Salz ein Cobalt-II-Salz ist, welches eine minimale Löslichkeit von etwa 0,01 Mol von Cobalt-II-Salz pro Liter Wasser bei 20°C (68°F) hat.

8. Verfahren gemäß irgendeinem der Ansprüche 5 bis 7, worin das Cobalt-II-Salz Cobaltacetat ist.

9. Verfahren nach Anspruch 5, worin die Cobaltkonversionslösung durch eine Badzusammensetzungs- bzw. Badauffüllungsfolge bzw. -sequenz hergestellt wird, umfassend:
(a) Auflösen des Metallcarboxylatsalzes, und
(b) dann Hinzufügen des Cobalt-II-Salzes.

10. Verfahren nach Anspruch 1, worin die Cobaltkonversionslösung einen pH von etwa 5,0 bis 9,0 hat.

11. Verfahren nach Anspruch 1, worin die Cobaltkonversionslösung eine Temperatur von etwa 20°C bis 71,1°C (68°F bis 160°F) hat.

12. Verfahren nach Anspruch 1, worin das Substrat mit der Cobaltkonversionslösung während einer Zeit von etwa 3 Minuten bis 60 Minuten kontaktiert wird.

13. Verfahren nach Anspruch 1, worin ein fluorinieries Benetzungsmittel zu der Cobaltkonversionslösung hinzugefügt wird, um die Bildung der Cobaltkonversionsbeschichtung auf dem Substrat zu unterstützen.

14. Verfahren nach Anspruch 13, worin das Benetzungsmittel aus der Gruppe ausgewählt ist, die folgendes umfaßt: Alkylfluorid, Fluorkohlenstoffe, CaF₂, MgF₂ und Mischungen hiervon.

15. Verfahren nach Anspruch 13, worin das Benetzungsmittel in der Menge hinzugefügt wird, die erforderlich ist, eine Flüssigkeiisoberflächenspannung von 0,03 bis 0,04 N/m (30 bis 40 Dyne pro Zentimeter) zu erzeugen.

16. Verfahren nach Anspruch 13, worin MgF₂, CaF₂ oder Mischungen hiervon zu der Lösung in einer Menge hinzugefügt wird bzw. werden, die im Bereich von 2 bis 4 Gramm pro Liter der endgültigen Lösung liegt.

17. Verfahren nach Anspruch 1, worin das Substrat Aluminium, Aluminiumlegierung, Magnesium, Magnesiumlegierung, Cd-plattiertes bzw. -galvanisiertes Substrat oder ein Zn-Ni-plattierzes bzw. -galvanisiertes Subtrat ist.

18. Gegenstand, der mittels des Verfahrens des Anspruchs 1 hergestellt ist.

19. Chemische Konversionbeschichtungslösung zum Erzeugen einer Oxidfilmcobaltkonversionsbeschichtung auf einem Metallsubstrat, wobei diese Lösung eine wäßrige Reaktionslösung umfaßt, welche einen löslichen Cobalt-III-hexakoordinierten Komplex enthält, der in der Form von Meₘ[Co(R)₆]ₙ vorhanden ist, worin Me eines oder mehrere ist bzw. sind, das bzw. die aus der aus Na, Li, K, Ca, Zn, Mg und Mn bestehenden Gruppe ausgewählt ist bzw. sind und worin m 2 oder 3 ist, n 1 oder 2 ist und R ein Carboxylat ist, das 1 bis 5 C-Atome hat, wobei die Konzentration des Cobalt-III-hexakoordinierten Komplexes von etwa 0,01 Mol pro Liter der Lösung bis zu der Sättigungsgrenze des Cobalt-III-hexakoordinierten Komplexes ist, wobei die wäßrige Reaktionslösung einen pH von etwa 5,0 bis 9,0 hat.

20. Lösung nach Anspruch 19, worin R Acetat ist.

21. Lösung nach Anspruch 19, worin der lösliche Cobalt-III-hexakoordinierte Komplex ein löslicher Cobait-III-Carboxylatkomplex ist, der durch Reagieren eines Cobalt-II-Salzes mit einem Metallcarboxylatsalz erhältlich ist, worin das Metall Me in Anspruch 19 definiert ist, welches 1 bis 5 C-Atome hat.

22. Lösung nach Anspruch 21, worin die Konzentration des Cobalt-II-Salzes von etwa 0,01 Mol pro Liter der endgültigen Lösung bis zu der Sättigungsgrenze des verwendeten Cobalt-II-Salzes ist und worin die Konzentration des Metallcarboxylatsalzes von etwa 0,03 bis 2,5 Mol pro Liter der endgültigen Lösung ist.

23. Lösung nach Anspruch 21, worin das Cobalt-II ein Cobalt-II-Salz ist, welches eine minimale Löslichkeit von etwa 0,01 Mol des Cobalt-II-Salzes pro Liter Wasser bei 20°C (68°F) hat.

24. Lösung nach Anspruch 21, worin das Cobalt-II-Salz Cobaltacetat ist.

25. Lösung nach Anspruch 21, worin das Metallcarboxylat ein Metallacetat ist.

26. Lösung nach Anspruch 21, worin die Cobaltkonversionslösung durch eine Badzusammensetzungs- bzw. Badauffüllungsfolge bzw. -sequenz hergestellt wird, umfassend:
(a) Auflösen des Metallcarboxylats; und
(b) dann Hinzufügen des Cobalt-II-Salzes.

27. Verwendung der Lösung des Anspruchs 19 zum Herstellen einer Oxidfilmcobaltkonversionsbeschichtung auf einem Metallsubstrat, worin die Lösung einen pH von etwa 5,0 bis 9,0 hat.

28. Verwendung der Lösung des Anspruch 19 zum Erzeugen einer Oxidfilmcobaltkonversionsbeschichtung auf einem Metallsubstrat, worin die Lösung eine Temperatur von etwa 20°C bis 71,7°C (68°F bis etwa 160°F) hat.

29. Verwendung der Lösung gemäß Anspruch 19 zum Herstellen einer Oxidfilmcobaltkonversionsbeschichtung auf einem Metallsubstrat, worin das Substrat Aluminium, eine Aluminiumlegierung, Magnesium, eine Magnesiumlegierung, Cd-plattiertes bzw. Cd-galvanisiertes Subtrat oder ein Zn-Ni-plattiertes bzw. -galvanisiertes Substrat ist.

30. Lösung nach Anspruch 19, umfassend ein fluozinieries Benetzungsmittel, das zu der Cobaltkonversionslösung hinzugefügt ist, um die Bildung der Cobaltkonversionsbeschichtung auf dem Substrat zu unterstützen.

31. Lösung nach Anspruch 30, worin das Benetzungsmittel ausgewählt ist aus der Gruppe, die folgendes umfaßt: Alkylfluorid, Fluorkohlenstoffe, CaF₂, MGF₂ und Mischungen hiervon.

32. Lösung nach Anspruch 30, worin das Benetzungsmittel in der Menge hinzugefügt ist, die erforderlich ist, um eine Flüssigkeitsoberflächenspannung von 0,C3 bis 0,04 N/m (30 bis 40 Dyne pro Zentimeter) zu erzeugen.

33. Lösung nach Anspruch 30, worin MgF₂, CaF₂ oder Mischungen hiervon zu der Lösung in einer Menge hinzugefügt sind, die im Bereich von 2 bis 4 pro Liter der endgültigen Lösung liegt.

## Revendications

1. Procédé pour la formation d'un revêtement de transformation au cobalt de film d'oxyde sur un substrat, dans lequel ledit substrat est de l'aluminium ou un alliage d'aluminium, ledit procédé comprenant les étapes consistant :
(a) à fournir une solution de transformation au cobalt formant un film d'oxyde comprenant une solution réactionnelle aqueuse comprenant un complexe hexacoordiné de cobalt-III soluble, dans lequel ledit complexe hexacoordiné de cobalt-III est présent dans la forme de Meₘ[Co(R)₆]ₙ, où Me est un ou plusieurs éléments choisis parmi Na, Li, K, Ca, Zn, Mg et Mn et où m est égal à 2 ou à 3, n est égal à 1 ou à 2 et R est un carboxylate ayant de 1 à 5 atomes de C, la concentration dudit complexe hexacoordiné de cobalt-III étant comprise entre environ 0,01 mole par litre de ladite solution réactionnelle aqueuse et la limite de saturation dudit complexe hexacoordiné de cobalt-III; et
(b) à mettre ledit substrat en contact avec ladite solution réactionnelle aqueuse sur une durée suffisante pour oxyder la surface dudit substrat, ledit revêtement de transformation au cobalt de film d'oxyde est par là formé, dans lequel ladite solution réactionnelle aqueuse présente un pH d'environ 5,0 à 9,0.

2. Procédé selon la revendication 1, dans lequel on ajoute un agent mouillant de fluorure d'alkyle ou de fluorocarbone à ladite solution réactionnelle aqueuse dans la quantité exigée pour produire une tension superficielle du liquide de 0,03 N/m à 0,04 N/m (30 à 40 dynes par centimètre).

3. Procédé selon les revendications 1 ou 2, dans lequel R est l'acétate.

4. Procédé selon les revendications 1, 2 ou 3, dans lequel la concentration dudit complexe hexavalent de cobalt-III est comprise entre environ 0,04 mole par litre de solution et environ 0,15 mole par litre de solution.

5. Procédé selon l'une quelconque des revendications 1-4, dans lequel ladite solution de transformation au cobalt est fournie en faisant réagir un sel de cobalt-II avec un carboxylate de métal ayant de 1 à 5 atomes de carbone.

6. Procédé selon la revendication 5, dans lequel la concentration dudit sel de cobalt-II est comprise entre environ 0,04 mole par litre de solution finale et environ 0,15 moles par litre de solution finale et la concentration du carboxylate de métal est comprise entre environ 0,03 et 2,5 mole par litre de solution finale.

7. Procédé selon les revendications 5 ou 6, dans lequel ledit sel de cobalt-II est un sel de cobalt-II qui présente une solubilité minimale d'environ 0,01 mole de sel de cobalt-II par litre d'eau à 20°C (68°F).

8. Procédé selon l'une quelconque des revendications 5-7, dans lequel ledit sel de cobalt-II est l'acétate de cobalt.

9. Procédé selon la revendication 5, dans lequel ladite solution de transformation au cobalt est préparée par une séquence de constitution du bain comprenant :
(a) la dissolution dudit sel de carboxylate de métal, et
(b) l'addition subséquente dudit sel de cobalt-II.

10. Procédé selon la revendication 1, dans lequel ladite solution de transformation au cobalt présente un pH d'environ 5,0 à 9,0.

11. Procédé selon la revendication 1, dans lequel ladite solution de transformation au cobalt présente une température d'environ 20°C à 71,1°C (68°F à 160°F).

12. Procédé selon la revendication 1, dans lequel ledit substrat est mis en contact avec ladite solution de transformation au cobalt sur une durée d'environ 3 minutes à 60 minutes.

13. Procédé selon la revendication 1, dans lequel on ajoute un agent mouillant fluoré à ladite solution de transformation au cobalt pour aider à la formation dudit revêtement de transformation au cobalt sur ledit substrat.

14. Procédé selon la revendication 13, dans lequel ledit agent mouillant est choisi parmi un fluorure d'alkyle, des fluorocarbones, CaF₂, MgF₂ et des mélanges de ceux-ci.

15. Procédé selon la revendication 13, dans lequel on ajoute ledit agent mouillant dans la quantité exigée pour produire une tension superficielle du liquide de 0,03 à 0,04 N/m (30 à 40 dynes par centimètre).

16. Procédé selon la revendication 13, dans lequel on ajoute MgF_{2,} CaF₂ ou des mélanges de ceux-ci à ladite solution dans une quantité comprise entre 2 et 4 grammes par litre de solution finale.

17. Procédé selon la revendication 1, dans lequel ledit substrat est de l'aluminium, un alliage d'aluminium, du magnésium, un alliage de magnésium, un substrat plaqué de Cd ou un substrat plaqué de Zn-Ni.

18. Article produit par le procédé selon la revendication 1.

19. Solution de revêtement de transformation chimique pour la production d'un revêtement de transformation au cobalt de film d'oxyde sur un substrat métallique, ladite solution comprenant une solution réactionnelle aqueuse comprenant un complexe hexacoordiné de cobalt-III soluble présent dans la forme de Meₘ[Co(R)₆]ₙ, où Me est un ou plusieurs éléments choisis parmi Na, Li, K, Ca, Zn, Mg et Mn et où m est égal à 2 ou à 3, n est égal à 1 ou à 2 et R est un carboxylate ayant de 1 à 5 atomes de C, la concentration dudit complexe hexacoordiné de cobalt-III étant comprise entre environ 0,01 mole par litre de solution et la limite de saturation dudit complexe hexacoordiné de cobalt-III, la solution réactionnelle aqueuse ayant un pH compris entre environ 5,0 et 9,0.

20. Solution selon la revendication 19, dans laquelle R est un acétate.

21. Solution selon la revendication 19, dans laquelle ledit complexe hexacoordiné de cobalt-III soluble est un complexe soluble de carboxylate de cobalt-III pouvant être obtenu en faisant réagir un sel de cobalt-II avec un sel de carboxylate de métal dans lequel le métal Me est défini dans la revendication 19 ayant de 1 à 5 atomes de C.

22. Solution selon la revendication 21, dans laquelle la concentration dudit sel de cobalt-II est comprise entre environ 0,01 mole par litre de solution finale et la limite de saturation du sel de cobalt-II utilisé et la concentration dudit sel de carboxylate de métal est comprise entre environ 0,03 et 2,5 mole par litre de solution finale.

23. Solution selon la revendication 21, dans laquelle ledit cobalt-II est un sel de cobalt-II qui présente une solubilité minimale d'environ 0,01 mole de sel de cobalt-II par litre d'eau à 20°C (68°F).

24. Solution selon la revendication 21, dans laquelle ledit sel de cobalt-II est l'acétate de cobalt.

25. Solution selon la revendication 21, dans laquelle ledit carboxylate de métal est un acétate de métal.

26. Solution selon la revendication 21, dans laquelle ladite solution de transformation au cobalt est préparée par une séquence de constitution du bain comprenant :
(a) la dissolution dudit carboxylate de métal; et
(b) l'addition subséquente dudit sel de cobalt-II.

27. Utilisation de la solution selon la revendication 19 pour la production d'un revêtement de transformation au cobalt de film d'oxyde sur un substrat métallique, dans laquelle ladite solution présente un pH d'environ 5,0 à 9,0.

28. Utilisation de la solution selon la revendication 19 pour la production d'un revêtement de transformation au cobalt de film d'oxyde sur un substrat métallique, dans laquelle ladite solution présente une température d'environ 20°C à 71,7°C (68°F à environ 160°F).

29. Utilisation de la solution selon la revendication 19 pour la production d'un revêtement de transformation au cobalt de film d'oxyde sur un substrat métallique, dans laquelle ledit substrat est de l'aluminium, un alliage d'aluminium, du magnésium, un alliage de magnésium, un substrat plaqué de Cd ou un substrat plaqué de Zn-Ni.

30. Solution selon la revendication 19 comprenant un agent mouillant fluoré ajouté à ladite solution de transformation au cobalt pour aider à la formation dudit revêtement de transformation au cobalt sur ledit substrat.

31. Solution selon la revendication 30, dans laquelle ledit agent mouillant est choisi parmi un fluorure d'alkyle, des fluorocarbones, CaF₂, MgF₂ et des mélanges de ceux-ci.

32. Solution selon la revendication 30, dans laquelle ledit agent mouillant est ajouté dans la quantité exigée pour produire une tension superficielle du liquide de 0,03 à 0,04 N/m (30 à 40 dynes par cm).

33. Solution selon la revendication 30, dans laquelle on ajoute MgF₂, CaF₂ ou des mélanges de ceux-ci à ladite solution dans une quantité comprise entre 2 et 4 g par litre de solution finale.
